

Sept. 1, 1931.

J. C. McFARLAND

1,821,561

METHOD OF DECORATING WATCH DIALS, ETC

Filed June 22, 1928

Fig. 1.



Fig. 2.



Fig. 3.



Fig. 4.



Fig. 5.



Fig. 6.



Fig. 7.



Fig. 8.

Inventor:

James C. McFarland,  
By his son, Lee, Christopher, Niles.  
Attest,

## UNITED STATES PATENT OFFICE

JAMES C. McFARLAND, OF FORT THOMAS, KENTUCKY, ASSIGNOR TO THE WADSWORTH WATCH CASE CO., OF DAYTON, KENTUCKY, A CORPORATION OF KENTUCKY

## METHOD OF DECORATING WATCH DIALS, ETC.

Application filed June 22, 1928. Serial No. 287,537.

The present invention relates particularly to a method of providing a watch dial, or the like, with a decorative surface; and the primary object is to provide an improved and simple method of this character which will enable improved results to be obtained with great facility.

The improved method is applicable, for example, to the production of a watch dial from a brass dial blank, the face surface of the dial being provided with metal platings of contrasting colors. For illustration, the body surface of the dial may be in silver, and the numerals and such other design as may be desired may appear in polished gold.

A preferred method of procedure is illustrated in the accompanying drawings, in which—

Fig. 1 illustrates a dial blank having a silver plating applied thereto; Fig. 2 illustrates a further step in which a gold plating is applied over the silver plating; Fig. 3 illustrates a further step in which a chromium plating is applied over the gold plating; Fig. 4 illustrates a further step in which a suitable resist design (which may correspond with numerals and other design features on the dial) has been applied to the chromium surface; Fig. 5 illustrates a further step in which the exposed areas of chromium plating have been removed; Fig. 6 illustrates a further step in which the resist design and portions of the gold have been removed, leaving the gold numerals, etc., protected by chromium plating; Fig. 7 illustrates a further step in which the chromium plating has been removed, leaving the silver surface and the gold numerals, etc.; and Fig. 8 illustrates a plan of the face of the dial.

One may start with a base metal blank, such as brass, or other base metal, or base metal alloy. If it be desired to have the numerals and other portions of a decorative design in gold upon a silver background, this may be accomplished in accordance with the following description, stated as a preferred method:

Silver plate the dial blank; polish (or otherwise finish) the silver plating; gold plate the surface of the silver plating; chro-

mium plate the surface of the gold plating; apply suitable resist to protect the numerals, name, and any other portions which are to appear in gold, such as the small dial of the second hand; remove the chromium plating over the unprotected areas, as by means of dilute hydrochloric acid, or dilute sulphuric acid; pumice off the gold from the exposed gold areas and, at the same time, remove the resist covering the numerals, etc.; and finally strip off the chromium plating which covers the numerals, etc. This may be done by means of dilute hydrochloric acid, for example, leaving the gold numerals and any other design in gold which may have been protected by the chromium plating. The gold numerals, etc., will possess a polished gold appearance, set off by a silver background.

The operation of pumicing off the exposed gold and the resist over the numerals, etc., will not affect the chromium plating which protects the numerals; and, finally, as stated above, the chromium may be stripped from the numerals, etc.

It is unnecessary to polish the gold plating before applying the chromium plating, as the gold will have a polished appearance in any event. If a polished effect is not desired, any other desired finish may be employed.

It is obvious that one may start with a silver dial-blank, instead of producing a silver-plated blank. Any precious metal plating may be used in lieu of silver. Silver has been selected in the example given as a color which contrasts with gold. However, platinum, white gold, or green gold, may be used.

Instead of pumicing or polishing the silver-plating, for example, the silver surface may be given a sand-blast finish, a satin finish, or the like.

The resist employed for protecting the chromium at the areas corresponding with the numerals, etc., may be applied in any suitable manner. One may, if desired, apply a light-sensitive coating to the chromium plating; photographically produce an image of the numerals, name, etc., in the coating; subject the coating to a developing operation

to remove the unreacted portions, thus leaving a resist over the numerals, name, etc.; and may then proceed to remove the chromium plating at the exposed areas.

5 Variations in the process within the scope of the invention will be made.

Referring to the figures in the drawings, A designates a blank, such as a dial blank; B designates a silver surface; C designates 10 a gold surface over the silver surface; D designates a chromium surface over the gold surface; E designates a suitable resist design, say a design which protects the numerals, name, and small second hand dial; and F 15 designates the finished dial.

It may be added that in the operation of pumicing off the gold and resist mentioned above, the chromium plating over the numerals, name, etc., is not abraded or affected 20 by the pumicing operation. Chromium plating is hard, resistant, and free from danger of tarnishing; hence, if desired, the chromium plating design may itself be allowed to remain as one of the contrasting 25 plating designs of the finished article. For illustration, at one stage in the process described above, a gold background is present, and the numerals, name, etc., appear as a chromium plating design. These are contrasting colors. Other ways of producing contrasting color designs may be used by 30 properly selecting the metals.

The foregoing detailed description has been given for clearness of understanding 35 only, and no unnecessary limitations should be understood therefrom, but the appended claims should be construed as broadly as permissible, in view of the prior art.

40 What I regard as new, and desire to secure by Letters Patent, is:

1. The method of producing a decorative design on a metal surface, which comprises: applying to a precious metal surface having a given color a precious metal plating of another color; applying a chromium plating; applying a suitable resist design to the chromium plating; removing the exposed chromium plating; and removing the first-mentioned plating at the exposed areas and the 45 resist which covers the protected areas of the chromium plating.

2. The method of producing a decorative design on a metal surface, which comprises: applying to a precious metal surface having a given color a precious metal plating of another color; applying a chromium plating; applying a suitable resist design to the chromium plating; removing the exposed chromium plating; removing the first-mentioned 50 plating at the exposed areas and the resist which covers the protected areas of the chromium plating; and finally removing the chromium plating at the areas formerly protected by the resist design.

65 3. The method of producing a decorative

design on a metal surface which comprises: applying a precious metal plating of given color to a base metal blank; applying another precious metal plating of contrasting color to the first-mentioned plating; applying a 70 chromium plating to the second-mentioned plating; applying a suitable resist design to the chromium plating; dissolving the chromium plating throughout the exposed areas; and removing the second-mentioned plating 75 and the resist design.

4. The method of producing decorative design on a metal surface which comprises: applying a precious metal plating of given color to a base metal blank; applying another 80 precious metal plating of contrasting color to the first-mentioned plating; applying a chromium plating to the second-mentioned plating; applying a suitable resist design to the chromium plating; dissolving the chromium plating throughout the exposed areas; removing the second-mentioned plating and the resist design; and finally removing the 85 remaining chromium plating.

5. The method of producing a decorative 90 design on a metal surface, which comprises: applying a precious metal plating to a base metal blank and giving to said plating a desired finish; applying a precious metal plating of contrasting color to said first-mentioned plating; applying a chromium plating to said second-mentioned plating; applying a suitable resist design to said chromium plating; removing the chromium plating at the exposed areas; removing the exposed second-mentioned plating and said resist design; 100 and removing the remaining chromium plating.

6. The method of producing a decorative 105 design on a metal surface, which comprises: applying to a surface of a given color a plating of another color; applying a chromium plating design upon said first-mentioned plating; removing the exposed portions of said first-mentioned plating while said chromium plating design serves as a resist; and removing said chromium plating design.

JAMES C. MFARLAND.

115

120

125

130